

Nov. 4, 1941.

R. FRANCHOT

2,261,516

PRODUCING SILICON AND ALLOYS

Filed March 18, 1939

2 Sheets-Sheet 1



Nov. 4, 1941.

R. FRANCHOT

2,261,516

## PRODUCING SILICON AND ALLOYS

Filed March 18, 1939

2 Sheets-Sheet 2



## UNITED STATES PATENT OFFICE

2,261,516

## PRODUCING SILICON AND ALLOYS

Richard Franchot, Washington, D. C.

Application March 18, 1939, Serial No. 262,717

17 Claims. (Cl. 75—135)

This invention relates to producing silicon and alloys; and it comprises a process of obtaining reduced silicon as a product in the utilization of carbonaceous fuels, including soft coal, and preferably with fixation of air nitrogen, wherein the coal, in admixture with siliceous matter and with alkali, is subjected to low temperature destructive distillation by being passed in countercurrent to a flow of initially very hot gases with recovery of volatile coal products, the carbonized residue carrying silica and alkali is contacted with a heated air blast to form rich producer gas and cyanide vapor with reduction of siliceous matter to molten metal which is recovered and wherein cyanide is condensed and separated from a major portion of the producer gases, the remaining portion of these gases being utilized for the destructive distillation of the coal and, most advantageously, the air blast heat being obtained by recuperation of sensible heat from the major portion of the producer gases after separation of the cyanide therefrom; and the invention further comprises a metallurgical blast furnace adapted for carrying on the above process, in which a hearth and bosh of the usual type having air tuyères for admitting the preheated blast is provided with a top or roof carrying a controlled hot gas outlet of relatively large cross-sectional area connected with a conduit leading to a condensing chamber and heat interchanger for preheating the blast, and in which a separated shaft section, provided at one end with fuel charging means and with a regulated gas outlet, communicates at the other end with the furnace bosh through the roof thereof; all as more fully hereinafter set forth and as claimed.

Silicon is usually made by reducing silica with carbon in the electric furnace. In the presence of metallic iron the product is ferrosilicon, a ferro alloy of silicon containing, typically, 50 to 75 per cent Si. Substantially pure silicon has been made in the electric furnace. These processes are as a rule relatively inefficient in the use of electric power. The cost of reducing silica in the electric furnace is rather high.

Silica can be and is reduced in the blast furnace to make high silicon pig iron, a content of about 15 per cent silicon in the pig iron being the usual practical commercial limit. The coke consumption in making high silicon pig or ferrosilicon in the blast furnace has been extremely high.

Quite recently a new demand for silicon has been created in connection with the production of alloy steel and for other metallurgical pur-

poses. Reduction of silicon from silica at a low cost has become an important commercial object. In effect, this reduction stores energy in the form of silicon which can be transported and utilized to develop heat in the exothermic oxidation of silicon to silica. For certain purposes silicon is a highly advantageous fuel. It has a calorific energy of 7100 centigrade units per pound which compares with 8100 units per pound of carbon. 5 Silicon has an advantage over carbon as a metallurgical fuel in that all of its energy is available in  $\text{SiO}_2$  formation while in forming CO from carbon as in usual metallurgical processes, only 30 per cent of its total energy is utilized.

15 This invention accomplishes, as one of the main objects, the storage of energy in the form of metallic or elemental silicon at an extremely low cost. The calorific energy of carbon and air oxygen is stored directly in the form of silicon, 20 reduced from silica in a blast furnace. Energy stored by this reduction of silica can be recovered and utilized by oxidizing the silicon back to silica.

One of the cheapest forms of energy is that obtained by oxidation of carbon with air. The cost 25 of carbon energy compares favorably with that of water power. In the present invention, energy obtained by burning carbon to CO, constituting some 30 per cent of the total calorific value of carbon, is stored directly in reduced silicon. This 30 direct storage has many advantages over the usual indirect procedure of converting carbon energy to electric energy and then employing (storing) the electrical energy by reducing silica to silicon.

Reduction of silica with carbon requires a high 35 temperature and absorbs much heat. According to authoritative data, the reaction



absorbs 140,000 calories of heat, or 5000 centigrade heat units per pound of silicon reduced. The heat for the reduction must be available at a high temperature, around 1500° C. or above. In other words, the reduction of 1 pound silicon from 2.14 pounds silica with 0.857 pound carbon requires 5000 centigrade units or pound-calories at 1500° C.

45 In the blast furnace, the heat developed by the highly heated air blast burning carbon to CO in the hearth of the furnace develops considerable heat which is available at the hearth temperature approximating 1500° C. On the basis of a pound of carbon burning under blast furnace conditions with 5.6 pounds air of a usual 50 moisture content, say 5 grains  $\text{H}_2\text{O}$  per cubic

foot of air, the heat developed may be estimated as follows:

|                                                              | Lb. cal. |
|--------------------------------------------------------------|----------|
| 1 pound carbon burning to CO                                 | 2430     |
| Sensible heat of 1 lb. carbon at 1500° C.                    | 650      |
| Sensible heat of air blast at 600-800° C.,<br>5.6 lbs.       | 950      |
|                                                              | <hr/>    |
|                                                              | 4030     |
| Less decomposition 0.055 lb. H <sub>2</sub> O at 3225<br>cal | 177      |
|                                                              | <hr/>    |
|                                                              | 3853     |

It may be noted that the heat development is equivalent to about 47.5 per cent of the total calorific value of the carbon, although only 30 per cent of this value is expended. Of this, however, some 2700 units are carried away in approximately 6.6 pounds of carbon monoxide and nitrogen, the gas formed in the gasification with air oxygen of each pound of carbon. This leaves some 1100 calories as the heat available per pound of carbon at 1500° C., with a quite ordinary blast temperature averaging 700° C. The available heat is some 13.5 per cent of the total carbon oxidation energy, or over 40 per cent of the heat obtained in oxidizing carbon to CO. It is noted that the available heat, called hearth heat, is for the most part obtained from the blast heat and that the sensible heat of the combustion gases at 1500° is about three times the blast heat.

It thus appears that the heat required to reduce a pound of silicon with carbon, 5000 calories, is equal to the heat available from the burning of about 4.5 pounds of carbon with some 25 pounds of air at a usual blast temperature of 700° C. (1300° F.). In making silicon from silica, the total theoretical consumption of carbon, including that oxidized by the silica, may be estimated as 5.4 pounds carbon per pound silicon. This can be lowered by increasing the blast heat. However, 600°-800° C. is a convenient range of blast temperatures.

In the blast furnace as at present constituted, consumption of coke in reducing silicon is considerably above the theoretical. For example, ordinary basic pig iron made from the richer Lake ores requires often less than a ton of coke per ton of pig. To make a pig iron containing 12 per cent silicon, or 14 per cent on the iron content, the coke consumption is usually more than doubled. In other words, reduction of 280 pounds silicon consumes about 1.12 tons of coke, or about 7 pounds carbon per pound silicon. This is some 30 per cent above the theoretical, as estimated.

I have discovered that the reduction of silicon can be accomplished under blast furnace conditions with nearly theoretical fuel economy, that is, by storage in silicon of not less than about 40 per cent of the energy set free in oxidizing carbon to CO with air oxygen, and 100 per cent of the carbon energy utilized in the oxidation of carbon by the silica reduced to silicon. To accomplish this I utilize for preheating the carbon and silica only a minor fraction of the gas produced by the air and obtain the blast heat by transferring sensible heat from a major fraction of the gas to the air blown into the furnace, which develops the hearth heat. Theoretically, it requires not more than a third of the sensible heat of the combustion gases to furnish the blast heat, and not more than a third to preheat the

carbon and silica. So operating, the "solution loss" of carbon in the furnace is prevented and substantially all of the carbon charged as fuel, except that which actually reacts with silica, is burned with air to develop heat.

The solution loss, gasification of carbon by CO<sub>2</sub> above the hearth, usually accounts for 15 to 25 per cent of the coke consumed in the blast furnace making pig iron. Solution loss is particularly severe in making the high silicon pig irons in the blast furnace. It is this action, CO<sub>2</sub>+C=2CO, which, to a considerable extent, determines the function of the blast furnace as a gas producer. In the present invention the solution loss reaction is under substantially complete control. The fixed carbon of the fuel may all be burned in the hearth of the furnace and oxidized to carbon monoxide by air and silica in a ratio of the order of 85:15. And, if desired, about 50 per cent of the energy of CO formation may be stored as silicon—about 15 per cent of the total calorific value of the carbon—leaving 70 per cent of the total value in the producer gas to be otherwise utilized. In other words, 30 per cent of the fuel value of carbon may be converted to silicon at an efficiency of 50 per cent, making silicon an inexpensive fuel. In effect, silica is utilized as "endothemic" in gasifying carbon with air to make producer gas.

I have further discovered in making silicon under blast furnace conditions that it is unnecessary to produce a great amount of slag. The silica needed may be supplied by the ash of the carbon fuel. A fuel may be chosen having sufficient ash content to furnish all the silicon to be reduced. All of the metallic oxides of the ash may be reduced to metal and in such case little or no slag is formed, all or the greater part of the silica of the ash being reduced to silicon. Ash composed of silica, iron oxide and alumina is reduced to a metallic alloy of silicon, iron and aluminum. By choosing a fuel carrying these oxides in proper proportions in the ash, a metal of desired composition can be produced. In this connection it is noted that storage of energy in the form of metallic aluminum to be used as a "thermite" fuel is the same in principle as production of silicon to be used as fuel. In the reduction of the fuel ash, when all or substantially all of the silica present is reduced, then alumina present is also reduced and the metal contains aluminum. Any iron oxide in the fuel ash is of course reduced in preference to the silica and, as I have found, silica is reduced in preference to alumina. When a ferrosilicon alloy or silicide is desired as the metal product, iron oxide may be added to the fuel charge or a fuel ash containing considerable iron oxide may be utilized. If ferrochrome silicon is wanted, an addition of chromite ore to the fuel charge results in adding chromium to the metal, the chromium oxide being reduced ahead of the alumina. Reduction of alumina can be controlled by having in the charge sufficient silica or other reducible oxide to absorb the available reducing energy, and a small excess of silica which may be slagged together with alumina present as an alumino-silicate slag. For this a little lime, fluorspar etc. can be added to the fuel charge to serve as fluxes. As stated however, it is possible to adjust the furnace charge so as to reduce considerable alumina and thus to obtain aluminum-silicon or ferroaluminum-silicon as the metal product.

I have further discovered in gasifying carbon with air and silica that the activity of the air

nitrogen at blast furnace temperatures can be utilized to advantage in promoting the reduction of silicon. Although generally regarded as an inert element, the actual fact is, nitrogen at 1500° C. reacts with many other elements, forming nitrides and carbonitrides. In particular, it is known that alkali cyanides are formed in considerable amounts in the blast furnace while making pig-iron. Cyanide formation is attributed to accumulation in the furnace of small amounts of potash, soda etc. contained in the ore and coke ash; the alkalis being driven from the slag by the action of lime, (which is used as flux) vaporized in the hearth and carried up the shaft where they are condensed. In the hearth, the alkalis react with carbon and air nitrogen, forming cyanide vapors in the gas. In the condensation in the cooler shaft, the cyanides are oxidized and revert to alkali oxides, returning with the slag to be again converted to cyanide vapors in the hearth. When it is considered that near 80 per cent of the air is nitrogen, that for every pound of carbon burning with air oxygen about 4.25 pounds of nitrogen are passed through the furnace, it is seen that the activity of nitrogen of 1500° C. is an important factor in the furnace economy. Nitrogen fixation always lowers the combustion temperature below the theoretical point. The furnace thus functions to a considerable extent as a reflux condenser.

In the present invention I take advantage of the nitrogen activity in cyanide formation by charging with the fuel to be gasified a substantial proportion of an alkali compound such as soda ash, sodium carbonate, potash, etc. The alkali first combines with the ash of the fuel as silicate (or aluminate) and in the hearth and bosh of the furnace is converted to cyanide vapor in a reaction which may be represented by the equation:



In this reaction silicon is produced in molten form and cyanide vapor goes forward with the gases formed from the air,  $2\text{CO} + 3.78\text{N}_2$ . The air gas is enriched in CO content by subtraction of nitrogen and addition of CO. A part of the heat generated by the air oxygen is taken up in cyanide vapor formation. It is noted that the above equation may be regarded as the sum of the two equations:



Reaction 3 is estimated to absorb 25,000 calories plus the heat of vaporization of 2 moles cyanide, estimated at 74,000 cal.; 893 cal. plus 2643 cal. per pound of nitrogen fixed as cyanide. It may be noted that the available combustion heat from a pound of carbon burning with air (blast heat 700° C.), 1100 cal., is about equal to the heat absorbed in fixing as cyanide vapor 0.3 lb. nitrogen or some 7 per cent of the air nitrogen; some 30 per cent nitrogen on the weight of the carbon burning with air, and over 20 per cent of the total carbon gasified exothermically by oxygen and endothermically by nitrogen.

Another and secondary reaction taking place as cyanide vapor contacts sodium silicate may be written:



silicon being formed together with sodium oxide

which reacts with carbon and nitrogen to form cyanide as in Equation 3. This reaction illustrates the strong reducing power of cyanide serving as a cyclic carrier of carbon in vapor and liquid form. Silica is reduced by cyanide formed in situ. Some tendency of the silicon to become nitrided is overcome by cyanide formation. When carbide-forming metals, aluminum, chromium, iron etc., are reduced together with the silicon, the carbides react with sodium and nitrogen to form metal and cyanide, thus giving low carbon metals. Cyanide and soda react together to form sodium:



Sodium vapor in the gases scavenges carbon and nitrogen from the reduced metals in cyanide formation. The fuel sulfur is for the most part carried out of the furnace as sulfur compounds, sulfo-cyanides, etc. in the hot gas.

One of the advantages of having alkali present to form cyanide during the reduction of silica in the blast furnace is to facilitate the production of a metal of high silicon content and having a low carbon content. In reducing the ash of the fuel to obtain high silicon alloys containing iron or iron and aluminum, the carbon content of the metal is kept well below 1 per cent and can be reduced to 0.1 per cent or less by cyanide formation from alkali charged with the fuel. The sulfur content of the metal is also kept low.

The net result of various reactions taking place at high temperatures in the hearth and bosh of the furnace is the production of enriched produced gas containing cyanide vapor and of clean metal. The relative proportions can be adjusted by variation of the amounts of soda and of silica (with other reducible oxides) charged with the fuel. The "burden" put upon the fuel consists of silicon and metal reduction and nitrogen fixation in a desired ratio. Cyanide is recovered by condensation of the vapor from the major portion of gases withdrawn directly and in a vertical direction from the furnace at the top of the bosh. The cyanide vapor in the minor fraction of the gases which is led through the furnace shaft to preheat the fuel charge is condensed and oxidized in the downwardly moving fuel charge, carried back to the hearth to be again converted to cyanide vapor, and eventually added to the cyanide recovered by condensation from the bosh gases.

In condensing cyanide from a major fraction of the gases produced in the hearth, it is advantageous to lead them through a mass of coke or other form of carbon impregnated with alkali (soda) and thus to lower the temperature and take up the latent heat of cyanide vapor in forming more cyanide in the liquid phase. The reaction,



absorbing 134,320 calories, or 4800 cal. per pound nitrogen, may be relied upon to take up the heat set free in the condensation of cyanide containing about 1.8 pounds nitrogen; which is to say that cyanide vapor in condensing to liquid supplies the heat to form from sodium carbonate over 50 per cent additional cyanide in the liquid phase. As I have found, the reaction goes forward with good velocity, the cyanide vapor in the gases not only supplying heat but also accel-

erating the decomposition of sodium carbonate to sodium by the reaction



The sodium as formed reacts exothermically in a formation of sodium cyanide from its elements. The gases carrying cyanide vapor thus may be cooled to about 1000°-1100° C. by formation of a 50 per cent increment of cyanide in the liquid phase.

In theory, according to the above estimates, it appears to be possible to fix as cyanide vapor about 7 per cent of the air nitrogen involved in gasifying carbon with heated air under blast furnace conditions; and in condensing the vapor to obtain a 50 per cent increment or a total fixation of 10 per cent of the air nitrogen. This estimate is, of course, based upon an assumption that all the high temperature available hearth heat is utilized in nitrogen fixation and that none is left for reduction of silicon and metals.

As a matter of fact, however, a primary fixation of 7 per cent of the air nitrogen, involving a charge with the fuel of 0.8 pound soda ash per pound carbon, would leave a deficiency of hearth heat available for reduction of silicon and the fuel might be overburdened by its own ash, however small in amount. Fixing 10 per cent of the air nitrogen means a production of more than a ton of cyanide per ton of fuel carbon gasified in the furnace.

A convenient and desirable operation includes use of a fuel of considerable ash content having a composition giving upon reduction metal of high silicon content, accompanied by fixation of 1 to 2 per cent of the air nitrogen. This involves charging with the fuel carbon about 20 per cent by weight of sodium carbonate and producing 300 to 600 pounds cyanide per ton of fuel carbon. A theoretical yield of reduced silicon equal to 18.5 per cent by weight of the fuel carbon suggests as a theoretical limit charging with the fuel carbon about 40 per cent silica or equivalent oxide to be reduced. A fuel containing 10 per cent siliceous ash by weight of the carbon absorbs about 25 per cent of the available heat in reducing its own ash. A low grade fuel of 34 per cent ash content leaves room for a primary fixation of 1 per cent of the air nitrogen which, with a secondary 50 per cent increment in condensation brings the total nitrogen fixation up to 1.5 per cent. Such an operation is entirely possible, yielding per pound of fuel carbon charged into the furnace 0.16 pound reduced silicon and 0.05 pound fixed nitrogen in the form of 0.17 lb. sodium cyanide. The ash of the carbon fuel is converted to a silicon fuel at the expense of a little over 30 per cent of the fuel value; and the byproducts (fixed nitrogen and good producer gas) are capable of paying for the operation. Thus silicon-metal is made available as an inexpensive metallurgical fuel derived from the ash of carbonaceous fuels.

The cyanide is readily converted by reaction with  $\text{H}_2\text{O}$  into ammonia and either formate, oxalate, or carbonate, depending upon the temperature. Any of these can be used cyclically to supply alkali to the furnace for fixation of air nitrogen as cyanide.

It is noted that both silicon reduction and nitrogen fixation, as described, effect considerable enrichment of the producer or air gas. Silicon reduction adds carbon monoxide to the normal air gas and nitrogen fixation as cyanide both adds CO and subtracts nitrogen. For example,

on the basis of 7 per cent primary fixation of air nitrogen as cyanide, the combustion reaction may be written:



When a further 3.5 per cent of the air nitrogen is fixed with soda ash according to Equation 6, each molecule of fixed nitrogen being replaced by 3 molecules of CO, the gas becomes



which is over 43 per cent carbon monoxide. Normal air gas runs about 35 per cent CO. The enriched producer gas is of course useful as fuel, particularly in gas engines operating generators of electric current.

In the process of storing a part of the energy of carbon directly in reduced silicon with or without aluminum, any solid carbonaceous material may serve as fuel. The ash, if any, is usually composed of  $\text{SiO}_2$ ,  $\text{Al}_2\text{O}_3$  and metallic oxides, which are converted to metal. Coke, as usual, serves excellently as carbon fuel. Ashless coke and silica rock may be used. However, further economy is possible by using raw bituminous coal of high volatile content. Low grade, high ash coals are advantageous. A mixture of coal and coke is sometimes advantageous. The coal is subjected to destructive distillation followed by carbonization in passing downward through the shaft in countercurrent to ascending hearth gases in regulated amounts. Liquid distillation products are readily recovered from the exit gases, and in addition coal gas of high calorific value may be produced if desired. Alkali charged with the coal aids in the distillation by increasing the proportion of hydrocarbons in both the liquid and gaseous distillation products. Thus the alkali is made to serve two purposes. Steam introduced part way up the shaft effects a hydrogenating action upon the coal. Hydrogen for this hydrogenating action can also be obtained by steaming the cyanide in the lower part of a furnace shaft, advantageously not far above the point where the separated shaft delivers into the bosh through its roof. Cyanide and steam at temperatures about 1000° react to form carbonate, hydrogen and nitrogen. By impregnating the coal with a hydrogenation catalyst the yield of lighter hydrocarbon oils is increased. For this, it is advantageous also to have alkali present with the coal in the hydroxide form. The distillation of the coal at controlled temperatures in the presence of caustic alkali and hydrogen formed from steam by reaction with cyanide, adds substantially to the value of the products of the process. In this, non-coking coals are used to advantage. The operation is controlled by regulating the proportion of the hearth gases passed through the shaft. A reserve of additional blast heat may be maintained.

It is advantageous to operate the process in connection with byproduct coke ovens at a steel plant where part of the rich producer gas produced in the process may be utilized for heating the coke ovens, thus making the coke oven gas fully available for use at the steel furnaces; the coke being utilized as fuel for production of silicon to serve as fuel in making steel direct from ore and scrap metal. With the coke used to produce silicon, a low grade high ash coal may be mixed to supply silica for reduction to silicon.

It is also advantageous to operate the process in conjunction with a coal mine for converting coal fuel to silicon fuel and producer gas with nitrogen fixation and recovery of valuable liquid fuel products from the coal. For this, cannel coal is particularly useful.

In the accompanying drawings I show more or less diagrammatically types of metallurgical blast furnaces within my invention and well adapted for carrying on the described process. In this showing,

Fig. 1 is a sectional view in elevation of one type of blast furnace, and

Fig. 2 is a similar view of a modified type of furnace.

Referring to Fig. 1, a blast furnace hearth and bosh 1 of usual construction is provided with a top cover or roof 2 of refractory material such as firebrick. The hearth has air-tuyères 3 supplied with preheated air from a surrounding bustle pipe 4 provided with suitable connecting members. A metal outlet 5 and slag outlet 6 are provided. A hot gas outlet 7 runs through the roof 2. A gas conduit 8 of refractory insulated material conveys hot gases from the hot gas outlet 7 to a condenser 10 adapted to condense cyanide vapor and to collect liquid cyanide as condensed from the hot gases. Advantageously a refractory nozzle member 9 terminates the conduit 8 and restricts the flow of gases through outlet 7, maintaining a pressure in the furnace. The nozzle may be water-cooled.

As shown, condenser 10 is provided with a bell and hopper 11 for charging carbon and soda in admixture into the condenser to serve as endothermic cooling agents for the hot gas aiding in condensation of cyanide vapor to the molten or liquid form. From the condenser in its lower portion, a gas conduit 12 leads to heat interchanger 13 which may be of a known metal or other suitable construction adapted to recuperate and transfer sensible heat from the gas to the air blast blown by blower 14 through the interchanger or recuperator to air conduit 15 leading to air bustle pipe 4. From the interchanger a gas conduit 17 provided with a valve 18 leads the cooled gas to a place of use (not shown) which may advantageously be a gas engine-generator plant for transforming producer gas into electric power. A small portion of this power is needed for operating blower 14.

The cyanide condenser 10 is shown as provided with a bottom outlet 20 for liquid cyanide. This outlet may deliver into a chamber 21 with a gas-tight connection, the chamber being provided with a valved inlet 22 for steam and water and a bottom outlet 23. A valved gas outlet 24 is also provided near the top of the chamber. A secondary tapping hole 25 is also shown in the bottom of the condenser.

The furnace shaft 27 communicates with the bosh and hearth through a shaft chute 28 which runs through the roof 2. The shaft 27 is shown supported by pillars 29, although any other convenient supporting means may be employed. At the top of the shaft a hopper and bell 30 serves to charge fuel into the furnace. Near the top of the shaft a gas outlet 31, controlled by valve 32 provides exit for gases passing from the furnace hearth up through the shaft. This gas outlet may run to a scrubber 33 where condensable products may be removed from the shaft gas to be collected as liquid in chamber 34. This chamber is shown provided with valved liquid outlets 35 and 36 at different levels and with gas outlet conduit 37,

having a valved branch 37a. The gas conduit is shown with a connection leading to boiler 38 and steam superheater 39, from which superheated steam may be run through pipe 40 to steam inlet 41 in the lower part of shaft 27. The shaft may be provided with a valved outlet 43 for carbonized material.

In Fig. 2 is shown a modified blast furnace having the hearth and bosh, hot gas outlet and appurtenances similar to those shown in Fig. 1. In the modified furnace, the shaft section comprises a horizontally inclined rotary kiln 45 operatively connected (by gears) to rotating means 46, such as a motor. The kiln is adapted to discharge into shaft chute 28, which communicates with the furnace bosh through cover 2. The kiln has a gas tight connection 47 at the lower end with chute 28, the latter having a closed cover 48 which may be made removable, if desired. At the upper end of the kiln, a vertical charging chamber 49 delivers into the kiln through a gas tight connection 50. Connections 47 and 50 may take the form of stuffing boxes. The charging bell hopper 51 and the valved gas outlet conduit 52 are similar in function to those shown in Fig. 1 (30 and 31). Steam inlets 53, 54 are shown in chute 28 which connects the horizontal furnace shaft to the bosh and hearth.

In operation, the two types of furnace function similarly, as will be clear in the following specific example of the process, in which a mixture of bituminous coals containing about 10 per cent ash is utilized. The ash analysis shows on the average 63 per cent  $SiO_2$ , 34 per cent  $Al_2O_3$ , 2 per cent  $Fe_2O_3$  with minor constituents which may be neglected. Upon reduction, this ash yields a metal containing about 61 per cent silicon, 35 per cent aluminum and 3 per cent iron. The coal mixture is non-coking and has an ultimate analysis of 5 per cent hydrogen, 6 per cent oxygen and 76 per cent carbon. Upon carbonization at a low red heat the coal yields 70 per cent fixed carbon and 20 per cent volatile matter.

A mixture of this coal with about 14 per cent by weight of sand or silica rock and 8 per cent by weight of soda ash is charged into the furnace through hopper 30 (or 51). The furnace may be started by first filling the hearth and bosh section 1 with coke and igniting the coke in the usual way under a cold air blast. As the coke burns away the products of combustion are divided, passing both through the condenser 10 to heat interchanger 13 and also up through shaft 27 (or 45) in predetermined proportions as controlled by valves 18 and 32 (or 52). As the furnace heats up with return in the air blast of sensible heat recuperated from the hot gas passing through outlet 7 to the heat interchanger, the coke is replaced in the bosh-hearth by the carbon-silica-soda residue left by countercurrent passage of hot gases and the coal mixture through the shaft. The hearth temperature soon rises to 1500° C. or thereabout. Gasification of this carbonized residue by action of the preheated air blast yields molten silicon metal which can be tapped through outlet 5. This metal is approximately 83 per cent Si, 15 per cent Al and 1 per cent Fe, little or no slag being formed in the furnace. By adding more silica to the furnace charge together with lime, fluorspar etc. as fluxes, the aluminum in the metal can be replaced by silicon, an alumino-silicate slag being formed and readily separated from the silicon. If ferro-silicon be desired as the metal product, a fuel with ash high in iron oxide con-

tent can be used or iron ore may be added to the furnace charge in the required proportion. If chrome-iron ore be used, a ferrochrome-silicon metal is obtained.

With the stated proportion of soda in the fuel charge, the combustion gases leaving the furnace bosh through the bosh gas outlet 7 carry sodium cyanide vapor in substantial proportions. Of the carbon residue passing through chute 28 into the bosh, and approximating 70 per cent by weight of the coal, some 13 to 14 per cent is used in reducing silica etc. and from 4 to 5 per cent is used in cyanide formation, leaving about 82 per cent (of the residue, or 55-60 per cent of the coal) to be gasified by air oxygen. In other words, say 13 per cent of the carbon reaching the hearth is gasified by silica, 82 per cent by air oxygen and 5 per cent by the air nitrogen and alkali. The fixation of nitrogen as cyanide vapor amounts to about one per cent of the air nitrogen.

Filling condenser 10 with lump coke impregnated with soda and charging coke and soda in proper proportions through the belled hopper 11 result in a further formation of cyanide in liquid form which, with that condensed from the gas, collects in the bottom of the condenser. The temperature of the gases in the condenser may thus be lowered to 1000 to 1100° C. The cyanide increment may amount to upwards of 50 per cent of that formed in the furnace hearth, bringing the total nitrogen fixed to around 1.5 per cent of the air nitrogen. Collected cyanide in molten form drops through outlet 20 into chamber 21. Other nitrogen compounds and condensable matter carried in the hot gas from the furnace are collected with the molten cyanide in condenser 10. Among these nitrogen compounds may be small quantities of a sodium silico-nitride or silico-cyanide. In chamber 21 the cyanide may be treated with the proper quantity of super-saturated steam admitted through pipe 22 to form formate and ammonia, this passing through outlet 24 to be collected and utilized. Molten cyanide can be tapped from the condenser as by means of tapping hole 25. The formate in chamber 21 may be recovered in aqueous solution passing through outlet 23. Formate crystallized from the solution may be utilized in various known ways. Or the solution may be recycled to the top of the furnace shaft and used to supply alkali for cyanide formation with recovery of hydrocarbons from the volatile matter of the coal.

In the carbonization of the coal passing downward through shaft 27 (or 45) by means of hot bosh gases passed upwardly in countercurrent through chute 28 a minor fraction of the gases formed in the hearth by gasification is sufficient. This leaves the greater part of the hearth gases to be utilized in recuperator 13 for supplying the blast heat needed for a blast temperature of 600 to 800° C. In some cases as little as 5 to 10 per cent of the bosh gases may suffice for the carbonization. In the described example superheated steam is admitted to the lower part of the shaft through inlet 41 (or 53 and 54). The steam reacts with cyanide carried up in the hearth gases and caught by the descending charge. Hydrogen is formed. The steam may also react with the carbon to form water gas, thus furnishing more hydrogen. As a result carbon compounds in the coal are hydrogenated and valuable liquid hydrocarbons are scrubbed

from the gases in scrubber 33 and collect in chamber 34.

In the example, utilizing the coal mixture specified, the following products are obtainable per ton of the coal charged into the furnace:

40 gallons hydrogenated tar oil

220 pounds silicon-metal

70 pounds fixed nitrogen

Producer gas containing 1400 pounds carbon.

The producer gas serves excellently for generation of electric power by gas-engine generators. At 25 to 30 per cent efficiency the producer gas is equivalent to over 1000 kilowatt hours per ton of coal. Also, it may be used to under fire coke ovens, or to dilute coke oven gas or natural gas before distribution.

In operating the furnace to utilize soft coal with destructive distillation and carbonization producing carbon for gasification in the hearth by a preheated air blast, fixing a substantial proportion of the air nitrogen and transforming the coal ash into a metallurgical fuel, it is possible to so operate the furnace shaft as to produce a good coal gas of high calorific power from the volatile matter of the coal. So operating, with careful regulation of temperatures in the furnace shaft, a coal carrying, say, over 30 per cent volatile matter and 60 per cent fixed carbon may be made to yield per ton, 20 to 30 gallons of tar and in addition some 3000 cubic feet of coal gas, 1000 to 1500 B. t. u. per cubic foot, this gas being diluted with producer gas utilized in the furnace shaft for distilling the coal. Thus utilization of coal according to the invention results in production of coal gas, oil, fixed nitrogen, electric power and silicon fuel.

In operating the process with raw coal as fuel, when the carbonization of the coal requires extended time for recovery of improved volatile products, the operation can be carried on in a blast furnace having more than one shaft supplying a single bosh hearth. For example, the furnace may have two or three chutes 28 each fed by a shaft 27 or rotary shaft 45 and a single hot gas outlet 7; this being usually sufficient.

In the process as described, silicon is reduced and air nitrogen fixed at the expense of 30 per cent of the calorific energy of fuel carbon. This is made possible by the sensible heat recuperation in the air blast; the quantity of heat available for work requiring high temperatures being determined by the blast temperature. The blast temperature can of course be raised and the yield of either silicon or fixed nitrogen or both be increased by burning some or all of the producer gas product in regenerative stoves and passing the air blast through such stoves on its way to the furnace. The yields of silicon and of fixed nitrogen are capable of being increased by enrichment of the air blast in oxygen. The yields can also be increased by utilizing in the furnace bosh electrical heat generated from the producer gas and applied by means of electrodes in known ways. However, from the standpoint of fuel efficiency, the direct transformation of fuel carbon to fuel silicon is highly advantageous.

What I claim is:

1. A continuous process of reducing silica to silicon which comprises gasifying carbon in admixture with silica in a blast furnace at about 1500° to 1600° C. with a blast of preheated air, passing a minor fraction of the gases thus produced in contact with the carbon-silica admixture to preheat the same preheating the air by re-

cuperation of sensible heat from a major fraction of said gases withdrawn from the furnace and removing from the zone of gasification a molten metal of high silicon content containing the greater part of the silicon of the silica admixed with the carbon.

2. A process of producing reduced silicon which comprises gasifying a carbon fuel containing a siliceous ash with a blast of preheated air in a blast furnace, preheating the carbon fuel by countercurrent contact with a regulated portion of the gases formed, preheating the air blast by recuperation of sensible heat from another regulated portion of said gases withdrawn from the furnace and recovering a metal containing most of the silicon of the fuel ash as a product of the process.

3. A process of reducing silica to silicon which comprises gasifying carbon under blast furnace conditions in the presence of silica and alkali at a temperature of about 1500° to 1600° C. with a blast of preheated air, thereby forming alkali cyanide vapor carried in gases produced from the air, reducing the greater part of the silica to silicon, recovering metal containing the reduced silicon in molten form, condensing cyanide from the gases and transferring sensible heat from the gases to the air blast.

4. A process of fixing air nitrogen with production of reduced silicon as a byproduct which comprises gasifying carbon under blast furnace conditions in a preheated mixture comprising carbonaceous fuel, silica and alkali with a blast of preheated air to produce reduced silicon in molten form and a gas containing nitrogen, carbon monoxide and alkali cyanide vapor, preheating said mixture with a minor fraction of the gases produced, recovering said reduced silicon as molten metal containing the greater part of the silicon of said mixture, condensing cyanide from a major fraction of said gases, and transferring heat from said major fraction to said air blast to preheat the same for silicon reduction.

5. In fixing nitrogen as alkali cyanide by gasification of carbon in the presence of alkali with preheated air, an improved process which comprises admixing silica with the carbon, gasifying the carbon under blast furnace conditions in predetermined proportions with air, alkali and silica respectively and recovering as a product of the process a metal containing reduced silicon as a major component.

6. A process which comprises converting the ash of a carbonaceous fuel into a metallurgical fuel by gasifying the fuel carbon under blast furnace conditions with preheated air and with alkali to reduce ash compounds to metal at the expense of a portion of the calorific energy of the carbon developed in CO formation, heat for said reduction being obtained in preheating the air for said gasification by recuperating heat from the air gases and fixed nitrogen compounds being recovered from said gases as a byproduct.

7. A continuous process of utilizing carbonaceous fuel containing siliceous ash which comprises gasifying the carbon of the fuel under blast furnace conditions with preheated air and with alkali to form carbon monoxide and alkali cyanide vapor while reducing the ash of the fuel to a silicon, containing metal and while preheating the fuel and alkali with a portion of said air gases and the air with a greater portion of said gases and recovering fixed nitrogen compounds from the latter portion of gases, thereby producing silicon-containing metal derived from the

fuel ash, fixed nitrogen and fuel gas as products of the process.

8. A process which comprises carbonizing soft coal containing ash by passing it in countercurrent to a flow of hot gases with recovery of volatile coal products from the exit gases, gasifying the carbonized coal under blast furnace conditions with preheated air, alkali and oxides of the ash in predetermined proportions, recovering metal containing silicon and aluminum reduced from the ash oxides and passing the gasification products in predetermined proportions to recuperate sensible heat in said air for gasification with recovery of alkali cyanide and to carbonize the coal, respectively.

9. A process of utilizing bituminous coal containing siliceous ash for production of coal volatiles, reduced silicon, fixed nitrogen and producer gas which comprises destructive distillation of said coal with addition of alkali by a flow of hot gases, forming said hot gases by gasifying the carbon residue under blast furnace conditions with a preheated air blast, recovering a metal containing reduced silicon derived from the ash of the coal and transferring sensible heat to the air blast from the greater part but not all of the gasification gases, alkali cyanide being recovered from said gases.

10. In recovering cyanide from hot producer gas carrying alkali cyanide vapor as formed by gasifying carbon under blast furnace conditions with preheated air, silica and alkali to reduce the silica, a process which comprises passing the major portion of gas into contact with carbon and alkali, thereby cooling the gas by endothermic formation of cyanide in the liquid phase, removing liquid cyanide from the gas and recuperating residual sensible heat from said gas in the air for said gasification, said recuperation of heat being quantitatively sufficient to effect reduction of the greater part of the silica.

11. In the fixation of air nitrogen as cyanide by gasification under blast furnace conditions of a siliceous ash-containing carbonaceous fuel with preheated air in the presence of alkali, a process improvement which comprises reducing silica of the fuel ash in the course of said gasification and withdrawing from the zone of gasification a molten silicon-containing metal reduced from said ash and containing a great part of the silicon of said ash.

12. In the fixation of air nitrogen as cyanide by gasification of a siliceous ash-containing carbonaceous fuel with preheated air in the presence of alkali, a process improvement which comprises gasifying under blast furnace conditions a carbonaceous fuel of relatively high ash content and withdrawing from the zone of gasification a molten metal containing silicon and aluminum reduced from said fuel ash.

13. In the fixation of air nitrogen as cyanide by gasification of a siliceous ash-containing carbonaceous fuel under blast furnace conditions with preheated air in the presence of alkali, a process of obtaining a silicon-containing metal as a product which comprises mixing silica with the fuel undergoing gasification and withdrawing from the zone of gasification a molten silicon-containing metal reduced from said ash and from said admixed silica.

14. A process of reducing silica to silicon in a blast furnace which comprises charging into the furnace a mixture of carbonaceous fuel with alkali and silica, heating the furnace with a blast of preheated air gasifying carbon of the

fuel and forming alkali silicate, reacting said silicate with carbon and the air nitrogen forming alkali cyanide and silicon, and recovering the silicon in molten metal form and the cyanide as products of the process.

15. In producing silicon alloys, a process of reducing silicon in a blast furnace which comprises reacting sodium silicate with sodium cyanide formed in situ in the blast furnace.

16. In producing silicon alloys, a process of reducing silicon in a blast furnace which comprises reacting sodium silicate with sodium cyanide formed in situ in the blast furnace and in the presence of producer gas and carbon.

17. A process of operating a blast furnace for production of metals which comprises adding alkali to the furnace charge of metal oxides and carbonaceous fuel, blowing the furnace with a blast of preheated air to provide high temperature heat in the furnace hearth maintaining in the hearth gases a substantial concentration of cyanide vapor formed from the added alkali and removing both reduced metal and alkali cyanide from the furnace.

RICHARD FRANCHOT.